

**G. W. SWIFT, JR.**  
**CORRUGATED PAPER BOARD AND PROCESS OF MAKING THE SAME.**  
**APPLICATION FILED DEC. 24, 1914.**

1,199,508.

Patented Sept. 26, 1916.

FIG. I.



FIG. II.



FIG. III.



FIG. IV.



FIG. V.



FIG. VI.



FIG. VII.



FIG. VIII



• WITNESSES:

WITNESSES.  
Frank E. Paige  
Philip W. Vessey.

**INVENTOR:**

INVENTOR:  
George W. Swift Jr.,  
by Arthur C. Page,  
Attorney.

# UNITED STATES PATENT OFFICE.

GEORGE W. SWIFT, JR., OF BORDENTOWN, NEW JERSEY.

## CORRUGATED PAPER-BOARD AND PROCESS OF MAKING THE SAME.

1,199,508.

Specification of Letters Patent. Patented Sept. 26, 1916.

Application filed December 24, 1914. Serial No. 878,891.

To all whom it may concern:

Be it known that I, GEORGE W. SWIFT, Jr., a citizen of the United States, residing at Bordentown, in the county of Burlington, in the State of New Jersey, have invented a certain new and useful Improvement in Corrugated Paper-Board and Processes of Making the Same, whereof the following is a specification, reference being had to the accompanying drawing.

My invention may be advantageously employed in producing cellular fabric including a corrugated paper web having a plane paper web attached upon one or both sides thereof. The corrugated web in such fabric, as ordinarily constructed, consists of either a single ply or a plurality of plies pasted together throughout their extent and attached to said plane web or webs by adhesive only applied thereto at the crests of its corrugations. Such fabric offers but slight resistance to crushing strains and is easily permanently collapsed, and, it is the object of my invention to produce a similar fabric which, for a given amount of paper employed therein, shall have greater capacity for resisting crushing strains, than said ordinary fabric, so that such a fabric of given strength may be made at less cost than the ordinary fabric aforesaid. My invention provides such a cellular fabric, wherein the corrugated web is reinforced, after it is corrugated, by a coating of primarily soluble nonfibrous material, which is more rigid but less costly than the paper of which said corrugated web is formed. As hereinafter described, such a coating is formed by an aqueous solution of sodium silicate which is conveniently sprayed upon the corrugated web and not only reinforces the latter upon its primarily plane face but serves as an adhesive for connecting the corrugated web with said plane web; which latter may be likewise reinforced by such a coating.

My invention includes the various novel features of construction, arrangement and procedure hereinafter more definitely specified.

In the drawing:—Figure I is a diagrammatic sectional view of mechanism whereby various fabrics embodying my invention may be produced. Figs. II to VII inclusive show, at successive stages of its formation, the constituent elements of a double plane faced fabric wherein only the corrugated

web is thus reinforced. Fig. II shows the primarily plane web which is first corrugated as shown in Fig. III, and then reinforced by a coating upon one surface as shown in Fig. IV. Fig. V shows said corrugated web attached at its upper crests to a plane web, and Fig. VI shows the fabric of Fig. V reinforced by a coating upon the opposite surface of said corrugated web. Fig. VII shows a second plane web attached to said fabric. Fig. VIII is a fragmentary edge view of a double plane faced fabric, such as shown in Fig. VII, but also having both of its plane webs reinforced by such coatings.

In said figures, the primarily plane web 1, which is to form the corrugated web, is directed between the intermeshed corrugated rollers 2 and 3 and thus corrugated as indicated at 4. Said corrugated web 4 is then reinforced with a coating of sodium silicate or other suitable material 5, conveniently sprayed thereon in aqueous solution, by means of the spraying device 6 under control of the valve 7. Before said coating has had time to dry upon said corrugated web 4 the latter is pressed into contact with the plane web 8 which is directed around the cylindrical roller 9, which may be spring 80 pressed toward said corrugated roller 3 which is preferably heated by steam introduced axially at 11, so as to dry the fabric during its passage around said roller 3, from which it is directed beneath the cylindrical 85 roller 13 which may be similarly heated by steam introduced axially at 14.

The procedure above described produces the fabric shown in Fig. V, consisting of the corrugated web 4 reinforced by the coating 5 upon one face thereof and connected with the single plane web 8, and such fabric may constitute a commercial product of my invention. However, the mechanism shown in Fig. I is adapted to produce a double 95 cellular fabric embodying my invention by providing the underface of said corrugated web 4 with the reinforcing coating 16 of sodium silicate, or other suitable material, conveniently sprayed thereon in aqueous solution by means of the spraying device 17 under control of the valve 18. Before said coating has had time to dry upon the lower face of said corrugated web 4, the latter is pressed into contact with the plane web 20 100 which is directed around the roller 21 which is opposed by the roller 22. Said rollers 21

and 22 are preferably heated by steam introduced axially therein respectively at 23 and 24, to insure that the reinforcing coating shall be dried in adhesion to the plane webs 8 and 20 to form the complete double fabric 25. Said rollers 21 and 22 are conveniently adjustable toward and away from each other and may be spring pressed so as to adapt them for fabric of different thicknesses.

The procedure above described provides the corrugated web 4, upon both faces, with respective reinforcing coatings 5 and 16 of uniform thickness throughout both faces of said web, and such coatings are sufficiently adhesive to retain the plane webs 8 and 20 as described. However, I find it convenient to include, in connection with the mechanism above described, means for providing the crests of the corrugations of said web 4 with additional adhesive material, and therefore provide the pasting devices including the receptacles 27 which may be supplied with sodium silicate solution, under control of the valves 28, or other suitable material which is picked up by the rollers 29 and distributed upon the web 4 by the rollers 30. Said rollers 29 and 30 may also be heated by steam introduced axially thereto. Moreover, said mechanism includes means for also providing the inner faces of said plane webs 8 and 20 with such coatings, including the spraying device 35 controlled by the valve 36 and the spraying device 38 controlled by the valve 39. By the employment of all of said spraying devices the cellular fabric shown in Fig. VIII is produced. Each of said spraying devices may conveniently include means for directing a blast of air in such relation to a passageway in communication with the liquid as to eject the latter into the blast, by which it may be atomized and thus sprayed. However, the specific construction of the spraying devices is not of the essence of my present invention, and any suitable form of device may be employed. However, I prefer to provide devices of the blast type aforesaid, in which hot air is employed so that the atomized solution shall be thus warmed.

I find it preferable to confine the spray from the spraying devices aforesaid by providing the latter with respective hoods 41 having walls extending transversely with respect to the webs, the full width of the latter, and end walls overlapping the edges of the respective webs as indicated.

Although I have shown the single tank 32 as the common source of supply of the adhesive solution to the several devices above described, it is to be understood that they may be otherwise supplied.

I do not desire to limit myself to the specific details of construction, arrangement or procedure herein set forth as it is obvious

that various modifications may be made therein without departing from my invention as defined in the appended claims.

I claim:

1. A corrugated paper board including outer plane webs and an intermediate corrugated web; said corrugated web being reinforced throughout its entire surfaces opposed to said plane webs, by an adherent coating of sodium silicate.

2. A corrugated paper board including outer plane webs and an intermediate corrugated web; said corrugated web being reinforced throughout its entire surfaces opposed to said plane webs, by an adherent coating of inorganic material; said coating being continuous throughout the extent of said corrugated web.

3. A corrugated paper board including outer plane webs and an intermediate corrugated web; said corrugated web being reinforced throughout its entire surfaces opposed to said plane webs, by an adherent coating of soluble material; said coating being continuous throughout the extent of said corrugated web.

4. A corrugated paper board including outer plane webs and an intermediate corrugated web; said corrugated web being reinforced throughout its entire surfaces opposed to said plane webs, by an adherent coating of nonfibrous material; said coating being continuous throughout the extent of said corrugated web.

5. A corrugated paper board including an outer plane web and a corrugated web; said corrugated web being reinforced upon both of its opposite surfaces by an adherent coating of sodium silicate.

6. A corrugated paper board including an outer plane web and a corrugated web; said corrugated web being reinforced upon its surface opposed to said plane web, by an adherent coating of sodium silicate.

7. A corrugated paper board including an outer plane web and a corrugated web; said corrugated web being reinforced upon both of its opposite surfaces by an adherent coating of inorganic material.

8. A corrugated paper board including an outer plane web and a corrugated web; said corrugated web being reinforced upon both of its opposite surfaces by an adherent coating of soluble material.

9. A corrugated paper board including an outer plane web and a corrugated web; said corrugated web being reinforced upon both of its opposite surfaces by an adherent coating of nonfibrous material.

10. A corrugated paper board including an outer plane web and a corrugated web; said corrugated web being reinforced upon its surface opposed to said plane web, by an adherent coating of inorganic material.

11. A corrugated paper board including

an outer plane web and a corrugated web; said corrugated web being reinforced upon its surface opposed to said plane web, by an adherent coating of soluble material.

5 12. A corrugated paper board including an outer plane web and a corrugated web; said corrugated web being reinforced upon its surface opposed to said plane web, by an adherent coating of nonfibrous material.

10 13. A corrugated paper web reinforced upon its surface by an adherent coating of sodium silicate extending between its crests and over the latter; more of said coating being applied at the crests than between

15 them.

14. The process of making a corrugated paper board, which consists in corrugating a primarily plane web; forming an adherent coating upon one face thereof, by spraying an aqueous solution of sodium silicate thereon; attaching a plane web to the coated side of said corrugated web; forming an adherent coating upon the opposite face of said corrugated web by spraying an aqueous solution of sodium silicate thereon; and attaching a plane web to the last coated side of said corrugated web.

20 15. The process of making a corrugated paper board, which consists in corrugating a primarily plane web; forming an adherent coating upon one face thereof, by spraying a liquid thereon; attaching a plane web to the coated side of said corrugated web;

25 forming an adherent coating upon the opposite side of said corrugated web by spraying a liquid thereon; and attaching a plane web to the last coated side of said corrugated web.

16. The process of making a corrugated paper board, which consists in corrugating a primarily plane web; forming an adherent coating upon one face thereof, by spraying an aqueous solution of sodium silicate thereon; and attaching a plane web to the coated side of said corrugated web.

30 17. The process of making a corrugated paper board, which consists in corrugating a primarily plane web; forming an adherent coating upon one face thereof, by spraying a liquid thereon; and attaching a plane web to the coated side of said corrugated web.

18. The process of making corrugated paper board which consists in corrugating a primarily plane web, forming a reinforcing coating by spraying adhesive liquid thereon, applying an additional coating of liquid to the crests of the corrugations, and attaching a plane web thereto.

In testimony whereof, I have hereunto signed my name at Bordentown, New Jersey, this seventeenth day of December, 1914.

GEORGE W. SWIFT, JR.

Witnesses:

WALTER ROBBINS,  
R. B. HOLLOWAY.